

## UNITED STATES PATENT OFFICE

LEON LILIENFELD, OF VIENNA, AUSTRIA

## PROCESS FOR IMPROVING VEGETABLE TEXTILE MATERIAL

No Drawing. Application filed June 16, 1927, Serial No. 199,410, and in Austria May 3, 1927.

It is known that by treatment with alkali and carbon bisulphide vegetable textile materials acquire valuable properties which, according to the conditions of treatment, find expression in a silky lustre or a finish, or in both (see German patent specification No. 129883, Austrian patent specifications Nos. 100194 and 101300 and British specifications Nos. 19912 of 1901, 1572 of 1915 and 168575).

10 The intensity of lustre which can be obtained by the processes hitherto used is, however, limited in degree, because if this degree is overstepped the thread or fabric under treatment becomes stiff, and thus loses its natural soft feel and is more or less hard and paper-like to the touch.

15 The present invention rests on the observation that particularly remarkable effects in respect of lustre or finish without deterioration of feel may be obtained by subjecting the fabric or yarn, which has been treated with alkali and carbon bisulphide, before it is brought into contact with an agent that precipitates viscose, to the action of a solvent 20 for cellulose xanthate.

25 If stretching be applied during the whole course of the process, or during that phase thereof which is suitable, there is obtained a silky lustre which exceeds considerably that obtainable by the usual mercerization process and at the same time the feel of the fabric or yarn is not substantially affected.

30 When the operation is conducted without any stretching, or the material allowed to shrink after or during the operation and the shrinkage is permitted to continue throughout the operation up to the finishing stage, or at least during a suitable phase of the operation, the fabric or yarn acquires a woolly condition.

35 Considering that the lustre obtainable with the aid of alkali and carbon bisulphide must be supposed to be due not only to the mercerizing effect of the alkali solution but also to the simultaneous effect of the carbon bisulphide, that is to say the conversion, at least superficially, of the yarn or fabric into cellulose xanthate, it is surprising that this lustre is not diminished or not appreciably 40 diminished by treatment with the solvent for

the cellulose xanthate. It remains uncertain whether this circumstance is to be attributed to an inhibition or weakening of the dissolving action of the solvent for cellulose xanthate by an intimate sorption between fibre 55 and viscose, or to a precipitation in part of the viscose formed within or on the fibre by any non-cellulosic substance contained in the fibre, that is to say the reconversion of such viscose into cellulose, or finally to the removal, together with the dissolved xanthate, of the outer layer of the fibre having adhering to it certain roughnesses which affect the lustre. 60

55 In carrying out the process the fabric or yarn which has been treated with alkali and carbon bisulphide is subjected, without first bringing it into contact with an agent which precipitates viscose with regeneration of cellulose, to the action of a solvent for cellulose xanthate. As suitable solvents may be named water or, preferably, a solution of a basic substance, such as caustic alkali or an alkali salt having an alkaline reaction, such as borax, an alkali sulphide, an alkali phosphate, an alkali acetate or an alkali carbonate, or a solution of an alkali sulphide in a caustic alkali solution, or a solution of a neutral salt which does not decompose viscose, such as common salt, or a dilute solution of an acid 70 which does not precipitate viscose, such as acetic acid or sulphurous acid. After the treatment with the solvent for cellulose xanthate the yarn or fabric may, optionally 75 after being washed, be brought into contact with any of the precipitating agents for viscose known in the viscose art and may then be washed and finished in known manner, or it may be directly washed and finished. 80

85 The following examples illustrate the invention, the parts being by weight:—

90 *Example 1.*—Bleached or unbleached cotton fabric or cotton yarn is treated in stretched condition with caustic soda solution of 18 to 22.5 per cent. strength at 15 95 to 20° C. and is then immediately, or after having remained a short or long time in the caustic soda solution (in some cases after removal of the excess of the caustic soda solution by pressing or centrifuging), sub- 100

jected to the action of carbon bisulphide vapour or of liquid carbon bisulphide either alone or mixed with a suitable diluent (for instance a solution of 0.5 to 10 per cent. 5 strength of carbon bisulphide in benzene) for a few seconds up to 10 minutes or longer, for example up to 2 to 5 hours. The yarn or fabric, in some cases after removal of the excess of carbon bisulphide by a current of air 10 or evacuation, is then brought into caustic soda solution of 5 to 18 per cent. strength at 15 to 18° C., or into an aqueous solution of sodium sulphide of 8 to 30 per cent. strength, or into a liquid containing 10 to 20 per cent. 15 of caustic soda and 10 per cent. of sodium sulphide, or into a solution of sodium carbonate of 10 per cent. strength, or into a dilute solution, say of 5 per cent. strength, of common salt. In the solvent for cellulose xanthate the yarn or fabric remains 20 for 5 minutes up to 2 hours, whereupon it is washed and then transferred to a bath which precipitates viscose. The latter may be any precipitating bath known in the viscose 25 art, for instance sulphuric acid of 10 per cent. strength or hydrochloric acid of 4 to 6 per cent. strength, or a solution of 4 parts of sodium bisulphate and 7 parts of sulphuric acid of 66° Baumé in 6 parts of water, or a 30 solution of 2 parts of ammonium chloride, 2 parts of sulphuric acid of 66° Bé. and 2 parts of glycerine in 14 parts of water, or a solution of 15 parts of sodium sulphate, 1 part of zinc sulphate, 7 parts of glucose and 35 8 parts of sulphuric acid of 66° Bé. in 69 parts of water. The precipitating bath may be used at room temperature or at raised temperature, such as 50° C. After the yarn or fabric has remained for a shorter or longer 40 time in the precipitating bath it is washed and dried.

Instead of a precipitating bath, another agent precipitating viscose, for example heat or steam may be employed.

45 Before or after the washing the yarn or fabric may be desulphurized in known manner, for example by treatment with a solution of sodium sulphide, or may be bleached, or may be treated by both operations.

50 The finished product is characterized by a highly silky lustre and an agreeable feel.

Example 2.—Mode of operation as in Example 1, with the difference that the fabric or yarn, after having been treated with the solvent for cellulose xanthate is, without being washed, transferred to the viscose precipitating bath.

Example 3.—The mode of operation is the same as in Example 1, with the difference that water is used as the solvent for cellulose xanthate.

Example 4.—The operation is the same as that in Example 1 or 2, with the difference 60 that the yarn or fabric, after it has been

treated with the solvent for cellulose xanthate, is only washed and dried.

Example 5.—The operation is the same as in Example 1, 2, 3 or 4, with the difference that the goods are not stretched during the 70 treatment with the caustic soda solution but only beginning with the treatment with carbon bisulphide.

Example 6.—The operation is the same as in Example 1, 2, 3, 4 or 5, with the difference 75 that the fabric or yarn is released from stretch before being washed.

Example 7.—The operation is the same as in Example 1, 2, 3, 4 or 5, with the difference 80 that the stretching is discontinued before drying.

In Examples 2, 3, 4, 5 and 7 the product is also a highly silky material of soft feel.

Example 8.—The operation is the same as in Example 1, 2, 3 or 4, with the difference 85 that the fabric or yarn is not stretched during the whole operation.

The result is a product which has a very full feel and woolly condition.

Example 9.—The operation is the same as 90 in Example 1, 2, 3, 4 or 5, with the difference that the stretching is discontinued before the treatment with the cellulose xanthate solvent. The result is a soft fabric or yarn of woolly character.

Example 10.—The operation is the same as in the foregoing examples, but with the difference that the mercerizing liquor contains only 9 to 12 per cent. of caustic soda.

Example 11.—Bleached or unbleached cotton fabric or cotton yarn is treated in stretched condition with undiluted carbon bisulphide or with carbon bisulphide diluted with benzene (for instance 1 to 5 parts of benzene to 1 part of carbon bisulphide) for a 100 few seconds up to a quarter of an hour. Then, if necessary, after expressing or centrifuging the excess of carbon bisulphide, the fabric or yarn is treated with caustic soda solution of 15 to 20 per cent. strength at room temperature for some minutes up to several hours. Further treatment occurs as described in Example 1, 2, 3 or 4.

Example 12.—The operation is the same as in Example 11, with the difference that 115 stretching is applied only after the treatment with carbon bisulphide.

Example 13.—The operation is the same as in Example 11, with the difference that the stretching is discontinued before introducing into the viscose precipitating bath.

Example 14.—The operation is the same as in Example 11, with the difference that the stretching is discontinued before drying.

The products obtained in accordance with Examples 11 to 14 are similar in appearance and feel to those obtained in Examples 1 to 6.

Example 15.—The operation is the same as in Example 11, with the difference that the 130

fabric or yarn is not stretched during the whole operation.

*Example 16.*—The operation is the same as in Example 11 or 12, with the difference that the stretching is discontinued before the treatment with the solvent for cellulose xanthate.

In Examples 15 and 16 there is obtained a yarn or fabric of woolly condition.

*Example 17.*—Bleached or unbleached cotton yarn or cotton fabric is treated in stretched condition with undiluted or diluted carbon bisulphide for several seconds up to 15 minutes. The fabric or yarn, if desired, after removal of the excess of carbon bisulphide by squeezing or centrifuging, is then brought into a caustic soda solution of 8 to 12 per cent. strength at 15 to 20° C. and is treated therein for some seconds up to 2 hours or even longer. The caustic soda solution in which the fabric or yarn is immersed is then cooled to 0° to -10° C. and kept at this temperature for some seconds up to 10 minutes. The further treatment is like that in Example 1, 2, 3 or 4.

*Example 18.*—The operation is the same as in Example 17, with the difference that the yarn or fabric after the treatment with carbon bisulphide is treated with caustic soda solution of 15 to 20 per cent. strength, for example of 18 per cent. strength, at 15 to 20° C. for several minutes up to 2 hours or even longer and is then brought into a caustic soda solution of 10 per cent. strength, cooled to 0° to -10° C. and allowed to remain therein for several seconds up to 10 minutes.

*Example 19.*—The operation is the same as in Example 17 or 18, with the difference that the stretching is applied after the treatment with carbon bisulphide.

*Example 20.*—The operation is the same as in Example 17 or 18, with the difference that the stretching is discontinued before the introduction into the viscose precipitating bath.

*Example 21.*—The operation is the same as in Example 17 or 18, with the difference that the stretching is discontinued before drying. The products obtained in accordance with Examples 17 to 21 are similar in respect to the appearance and feel to those obtained in accordance with Examples 1 to 6.

*Example 22.*—The operation is the same as in Example 17 or 18, with the difference that the fabric or yarn is not stretched during the whole operation.

*Example 23.*—The operation is the same as in Example 17, 18 or 19, with the difference that the stretching is discontinued before the treatment with the solvent for cellulose xanthate.

In Examples 22 and 23 there is obtained a yarn or fabric of woolly condition.

The cotton fabric or yarn treated in accordance with the invention, may be in the raw condition or preliminarily treated (for example boiled or keired by any known meth-

od), wetted or not wetted, mercerized or not mercerized. It may also be preliminarily treated with a hydrolyzing or gelatinizing agent, for instance a strong mineral acid, such as sulphuric acid of 49° to 60° Bé., or phosphoric acid of 55 to 57° Bé., or over, or hydrochloric acid of 24° Bé., or nitric acid of 43 to 46° Bé. or over, or hot zinc chloride solution of 60° Bé., or cupric oxide ammonia solution of high concentration.

The expression "vegetable textile material" in the specification and in the claims includes wherever the context permits, all vegetable textile materials, such as flax, linen, hemp, ramie-fibre, jute and particularly cotton and the like, in the form of pure vegetable fabrics (for example pure cotton fabrics) or mixed fabrics or in the form of yarn in skeins, cops, or warps.

The finished products may be calendered, schreinered, beetled or similarly treated.

The production of patterned effects by use of reserves is an obvious procedure.

I claim.

1. The process of improving the lustre or finish of vegetable textile material which has been treated with caustic alkali and carbon bisulphide to form cellulose xanthate which comprises subjecting the said so treated material to the action of a solvent for cellulose xanthate before it is subjected to the action of an agent capable of precipitating viscose.

2. The process of improving the lustre or finish of vegetable textile material which has been treated with caustic alkali and carbon bisulphide under conditions forming cellulose xanthate which comprises subjecting the said so treated material to the action of an agent which is a solvent for the cellulose xanthate so formed, the said so treated material being subjected to said agent before the said so treated material is subjected to an agency capable of regenerating cellulose from cellulose xanthates.

3. The process of improving vegetable textile material which has been subjected to the action of caustic alkali solution and carbon disulphide which comprises subjecting the so treated material, before it is subjected to an agency regenerating cellulose, to the action of a basic substance capable of dissolving cellulose xanthate.

4. The process of improving vegetable textile material which has been subjected to the action of caustic alkali solution and carbon bisulphide which comprises subjecting the so treated material, before it is subjected to an agency regenerating cellulose, to the action of a solution containing caustic alkali in such concentration as to be capable of dissolving cellulose xanthate.

5. The process of improving vegetable textile material which has been subjected to the action of caustic alkali solution and carbon bisulphide which comprises subjecting the

so treated material, before it is subjected to an agency regenerating cellulose, to the action of a solution containing caustic alkali and alkali sulphide in such concentrations as 5 to be capable of dissolving cellulose xanthate.

6. The process of improving the lustre or finish of vegetable textile material which comprises subjecting said material to the action of carbon bisulphide and caustic alkali, 10 and thereafter, before treatment with an agent capable of regenerating cellulose from viscose, subjecting the said treated material to the action of a solvent for cellulose xanthate.

15 7. The process of improving the lustre or finish of vegetable textile material which comprises converting it superficially into cellulose xanthate and before treatment with an agent capable of regenerating cellulose from 20 cellulose xanthate subjecting the said superficially converted material to the action of a solvent for cellulose xanthate.

8. The process of improving vegetable textile material which comprises converting it at 25 least superficially into cellulose xanthate and before subjecting it to an agency capable of regenerating cellulose from cellulose xanthate subjecting the so converted material to the action of a solvent for cellulose xanthate in 30 a step separate from the step of conversion into cellulose xanthate.

In testimony whereof I have hereunto set my hand.

LEON LILIENFELD.

35

40

45

50

55

60

65